

S. M. BULLOCK & H. S. LLOYD.

ABRASIVE,

APPLICATION FILED MAY 18, 1914.

1,133,260.

Patented Mar. 30, 1915.



WITNESSES

Victor Silgander

Charles F. T. Jr. By

Inventors  
Samuel M. Bullock.  
Harry S. Lloyd.  
Charles W. Field Atty

# UNITED STATES PATENT OFFICE.

SAMUEL M. BULLOCK, OF CHICAGO, AND HARRY S. LLOYD, OF OAK PARK, ILLINOIS.

## ABRASIVE.

1,133,260.

Specification of Letters Patent. Patented Mar. 30, 1915.

Application filed May 18, 1914. Serial No. 839,212.

*To all whom it may concern:*

Be it known that we, SAMUEL M. BULLOCK and HARRY S. LLOYD, citizens of the United States, and residents of the city of Chicago, in the county of Cook and State of Illinois, and of the village of Oak Park, in the county of Cook and State of Illinois, respectively, have invented certain new and useful Improvements in Abrasives; and we do hereby declare that the following is a full, clear, and exact description of the same, reference being had to the accompanying drawings, and to the numerals of reference marked thereon, which form a part of this specification.

There are a number of ways and means of constructing abrasive or grinding wheels, but many of these involve a tedious or involved process, while on the other hand those wheels capable of being manufactured in a simplified manner, have often proved unreliable for the purpose.

This invention relates to an exceedingly simple process for coating metal, wood, fiber, composition or fabric with an abrasive, enabling a grinding element, such as a wheel, disk or belt to be constructed or refinished by an inexperienced person and in a short space of time.

It is an object of this invention to provide a means of associating an abrasive with any suitable article by first coating or painting the article with a thin covering of liquid, then spreading or rubbing in a slight amount of a cement powder and finally spreading thereover a mixture of the abrasive and the powder which has been thoroughly mixed and wetted with the liquid.

It is furthermore an object of this invention to provide a means of applying an abrasive substance to an article by coating a fabric with a cementitious substance, and spreading thereon a mixture of abrasive and cement, and then applying the fabric to the article by means of the cement or any other suitable means.

It is finally an object of this invention to provide an improved simplified process for applying an abrasive to an article.

The invention (in a preferred form) is illustrated in the drawings and hereinafter more fully described.

In the drawings: Figure 1 is a front face view of an abrasive wheel constructed ac-

cording to our invention. Fig. 2 is a section on line 2—2 of Fig. 1.

As shown in the drawings, a disk, which may be either metal, wood, composition or fiber, is denoted by the reference numeral 1, and has rigidly secured on one face thereof a bearing collar 2, by means of screws 3. Both surfaces of the disk 1, are coated with an abrasive, although in a different manner.

Referring first to the means for applying the abrasive on the top surface of the disk shown in Fig. 2, or the surface opposite to that on which the bearing collar 2, is secured, the surface is first coated or wetted with a solution which consists of approximately 14.5% water and 85.5% magnesium chlorid. The wetted surface is then sprinkled with a cement powder known as calcined magnesite, which is rubbed in. An analysis of the powder shows:

|                     |       |
|---------------------|-------|
| Water               | 70%   |
| Calcium carbonate   | 16.05 |
| Magnesium carbonate | 2.38  |
| Magnesium oxid      | 75.87 |
| Silica              | 5.00  |

The abrasive mixture consists of emery, carborundum, alundum, aloxite, adamite, or any other well known abrasive substance and the magnesite, the proportions of which may vary for different purposes, for example for grinding gray iron castings two parts by volume of the abrasive are mixed with one part of the calcined magnesite powder. After thoroughly mixing these enough of the magnesium chlorid solution is added to make the whole like wet sand, and the wet mixture 4, is then packed upon the previously treated surface of the article. On the opposite surface of the disk we have shown the abrasive applied in a slightly different manner, and for this purpose a piece of fabric 5, is first treated with the magnesium chlorid solution and then a slight amount of the calcined magnesite powder is applied thereon, after which a mixture of the powder and abrasive in the proportion of one to two, or any desired proportion, as before described, is spread upon the fabric. This may be allowed to thoroughly dry, and may then be applied to the disk at any subsequent time, or may be applied immediately, and if so, the surface of the disk is wetted with the magne-

85  
90  
95  
100  
105  
110

sium chlorid solution as before, and coated with the magnesite powder, after which the coated fabric is applied, of course with the coated surface of the fabric faced outwardly.

It is obvious that the various sequence of operations for applying the abrasive substance to an article may be varied through a wide extent without departing from the principles of this invention. We therefore do not purpose limiting the patent granted otherwise than necessitated by the prior art.

We claim as our invention:

1. An abrasive coating comprising an abrasive intermixed with a magnesite ce-

ment adapted to be applied on an article previously treated with magnesium chlorid solution and dry calcined magnesite powder.

2. A cémentitious abrasive coating comprising a mixture of a magnesite cement and an abrasive in a ratio of one to two and magnesium chlorid solution.

In testimony whereof we have hereunto subscribed our names in the presence of two subscribing witnesses.

SAMUEL M. BULLOCK.  
HARRY S. LLOYD.

Witnesses:

LAWRENCE REIBSTEIN,  
FRANK K. HUDSON.